



US009005714B2

(12) **United States Patent**  
**Doessel et al.**

(10) **Patent No.:** **US 9,005,714 B2**  
(45) **Date of Patent:** **Apr. 14, 2015**

(54) **PROCESS FOR THE PRODUCTION OF A DARK-COLOR MULTI-LAYER COATING**

(75) Inventors: **Karl-Friedrich Doessel**, Wuppertal (DE); **Gunter Richter**, Wuppertal (DE)

(73) Assignee: **Axalta Coating Systems IP Co., LLC**, Wilmington, DE (US)

(\*) Notice: Subject to any disclaimer, the term of this patent is extended or adjusted under 35 U.S.C. 154(b) by 460 days.

(21) Appl. No.: **13/504,490**

(22) PCT Filed: **Oct. 27, 2010**

(86) PCT No.: **PCT/US2010/054266**

§ 371 (c)(1),  
(2), (4) Date: **May 21, 2012**

(87) PCT Pub. No.: **WO2011/056646**

PCT Pub. Date: **May 12, 2011**

(65) **Prior Publication Data**

US 2012/0269965 A1 Oct. 25, 2012

**Related U.S. Application Data**

(60) Provisional application No. 61/255,315, filed on Oct. 27, 2009.

(51) **Int. Cl.**

**B05D 7/16** (2006.01)  
**B05D 7/14** (2006.01)  
**B05D 7/00** (2006.01)  
**B05D 5/06** (2006.01)  
**B05D 1/02** (2006.01)

(52) **U.S. Cl.**

CPC **B05D 7/14** (2013.01); **B05D 7/572** (2013.01);  
**B05D 5/06** (2013.01); **B05D 7/16** (2013.01);  
**B05D 1/02** (2013.01)

(58) **Field of Classification Search**

None

See application file for complete search history.

(56)

**References Cited**

**U.S. PATENT DOCUMENTS**

8,722,150 B2 \* 5/2014 Richter et al. .... 427/407.1  
8,784,941 B2 \* 7/2014 Richter et al. .... 427/407.1  
8,835,008 B2 \* 9/2014 Richter et al. .... 428/411.1  
2010/0186891 A1 \* 7/2010 Ruch et al. .... 156/272.8  
2011/0070427 A1 \* 3/2011 Richter et al. .... 428/328  
2011/0070455 A1 \* 3/2011 Richter et al. .... 428/457  
2011/0171375 A1 \* 7/2011 Richter et al. .... 427/160  
2011/0195180 A1 \* 8/2011 Richter et al. .... 427/160  
2012/0269965 A1 \* 10/2012 Doessel et al. .... 427/160  
2012/0269975 A1 \* 10/2012 Doessel et al. .... 427/380  
2013/0276950 A1 \* 10/2013 Richter .... 156/60

\* cited by examiner

*Primary Examiner* — William Phillip Fletcher, III

(74) *Attorney, Agent, or Firm* — Ingrassia Fisher & Lorenz, P.C.

(57) **ABSTRACT**

A process for the production of a dark-color multi-layer coating, comprising the successive steps:

(1) applying an NIR-opaque coating layer A' from a solventborne coating composition A to a substrate,  
(2) applying a coating layer B' from a solventborne coating composition B onto the substrate provided with coating layer A',  
(3) subjecting the coated substrate obtained in step (2) to a drying step,  
(4) applying a clear coat layer, and  
(5) curing the coating layers simultaneously;  
wherein both coating compositions A and B comprise binders and crosslinkers comprising melamine-formaldehyde resin crosslinker,  
wherein both coating compositions A and B comprise certain proportions of cellulose ester binder and NAD binder and/or sheet silicate and/or fumed silica and/or urea SCA and/or polyolefin wax,  
wherein the pigment content of coating composition A consists 90 to 100 wt. % of aluminum flake pigment and 0 to 10 wt. % of further pigment,  
wherein the pigment content of coating composition B consists 50 to 100 wt. % of black pigment with low NIR absorption and 0 to 50 wt. % of further pigment.

**14 Claims, No Drawings**

## 1

## PROCESS FOR THE PRODUCTION OF A DARK-COLOR MULTI-LAYER COATING

## FIELD OF THE INVENTION

The invention is directed to a process for the production of a dark-color multi-layer coating.

## DESCRIPTION OF THE PRIOR ART

Dark-color coatings often contain carbon black pigments which absorb radiation in the near-infrared wavelength range and transform it into heat. Substrates coated with paint coatings of this type heat up in the NIR-containing sunlight; this occurs via heat conduction, i.e., heat is directly transferred to the substrate from the coating layer containing carbon black pigments and heated by solar radiation. This type of heating is often undesirable; for example, it may be undesirable for the actual substrate material itself and/or for the interior of the substrate to be heated up. Motor vehicles are probably the most prominent examples of substrates which comprise an interior. Vehicles with light-color coatings do not heat up as much and less fuel is required to operate the vehicle air-conditioning system than in corresponding models painted in a dark color.

US 2008/0187708 A1 discloses a dark color multi-layer coating comprising a first IR-reflecting layer comprising IR-reflective pigments in a resinous binder, and a second visible radiation absorbing layer with dark color being substantially transparent to IR radiation comprising a tint in a resinous binder comprising nano-sized pigments with an average primary particle size of up to 100 nm.

## SUMMARY OF THE INVENTION

It has been found that substrates with dark-color multi-layer coatings which heat up only comparatively slightly in sunlight may be produced using the wet-on-wet-on-wet coating process described hereinafter.

The invention is directed to a process for the production of a dark-color multi-layer coating, comprising the successive steps:

- (1) applying an NIR-opaque coating layer A' from a solvent-borne pigmented coating composition A to a substrate,
- (2) applying a coating layer B' from a solventborne pigmented coating composition B onto the substrate provided with coating layer A',
- (3) subjecting the coated substrate obtained in step (2) to a drying step,
- (4) applying a clear coat layer from a clear coat composition onto the coated substrate obtained in step (3), and
- (5) thermally curing the coating layers applied in steps (1), (2), and (4) simultaneously;

wherein both coating compositions A and B comprise resin solids consisting of binder solids plus crosslinker solids comprising melamine-formaldehyde resin crosslinker, wherein coating composition A comprises at least one component selected from the group consisting of (i) (a) >5 to 20 wt. % (weight-%) of cellulose ester binder and up to 10 wt. % of NAD (non-aqueous dispersion) binder or (b) 10 to 100 wt. % of NAD binder and up to 5 wt. % of cellulose ester binder, the wt. % in each case being based on the weight of the binder solids of coating composition A, (ii) 0.2 to 1.5 wt. %, based on the weight of the resin solids of coating composition A, of sheet silicate (layered silicate), (iii) 0.5 to 2 wt. %, based on the weight of the resin solids of coating composition A, of fumed silica (pyrogenic

## 2

silica), (iv) 0.5 to 2.5 wt. %, based on the weight of the resin solids of coating composition A, of urea SCA (sag control agent) and (v) 0.5 to 8 wt. %, based on the weight of the resin solids of coating composition A, of polyolefine wax,

- 5 wherein coating composition B comprises at least one component selected from the group consisting of (i') (a) >5 to 20 wt. % of cellulose ester binder and up to 10 wt. % of NAD binder or (b) 10 to 100 wt. % of NAD binder and up to 5 wt. % of cellulose ester binder, the wt. % in each case being based on the weight of the binder solids of coating composition B, (ii') 0.2 to 1.5 wt. %, based on the weight of the resin solids of coating composition B, of sheet silicate, (iii') 0.5 to 2 wt. %, based on the weight of the resin solids of coating composition B, of fumed silica, (iv') 0.5 to 2.5 wt. %, based on the weight of the resin solids of coating composition B, of urea SCA and (v') 0.5 to 8 wt. %, based on the weight of the resin solids of coating composition B, of polyolefine wax,
- 10 wherein the pigment content of coating composition A consists 90 to 100 wt. % of at least one aluminum flake pigment and 0 to 10 wt. % of at least one further pigment, which is selected in such a way that NIR-opaque coating layer A' exhibits low NIR absorption,
- 15 wherein the pigment content of coating composition B consists 50 to 100 wt. % of at least one black pigment with low NIR absorption and 0 to 50 wt. % of at least one further pigment, which is selected in such a way that coating layer B' exhibits low NIR absorption and that the dark-color multi-layer coating exhibits a brightness L\* (according to CIEL\*a\*b\*, DIN 6174), measured at an illumination angle of 45 degrees to the perpendicular (surface normal) and an observation angle of degrees to the specular (specular reflection), of at most 10 units.

In a particular embodiment of the process of the present invention, the at least one aluminum flake pigment forming 90 to 100 wt. % of the pigment content of coating composition A is selected among 10 to 80 nm thick aluminum flake pigments.

Apart from the pigmentation of both coating compositions A and B, it is also essential in the practice of the present process that coating composition A comprises at least one component selected from the group consisting of components (i) to (v) and that coating composition comprises at least one component selected from the group consisting of components (i') to (v'). It has been found that the presence of at least one component selected from the group consisting of components (i) to (v) in coating composition A and of at least one component selected from the group consisting of components (i') to (v') in coating composition B allows to achieve both, the desired dark-color shade of the multi-layer coating and the desired low heat development in sunlight, although coating compositions A and B and the clear coat composition are applied wet-on-wet-on-wet.

As already said, it is possible to select a combination of more than one component from the group consisting of components (i) to (v) when formulating coating composition A and a combination of more than one component from the group consisting of components (i') to (v') when formulating coating composition B. In such case, the skilled person will select the wt. % proportion of each component carefully and will in general not select the wt. % proportion of each component at the upper end of each component's wt. % range.

It is preferred that the at least one component selected from the group consisting of components (i) to (v) and contained in coating composition A is of the same type as the at least one component selected from the group consisting of components (i') to (v') and contained in coating composition B. For

example, if coating composition A contains NAD binder in a certain proportion within the range of 10 to 100 wt. %, based on the weight of the binder solids of coating composition A, and sheet silicate in a certain proportion within the range of 0.2 to 1.5 wt. %, based on the weight of the resin solids of coating composition A, it is preferred that coating composition B also contains NAD binder in a certain proportion within the range of 10 to 100 wt. %, based on the weight of the binder solids of coating composition B and sheet silicate in a certain proportion within the range of 0.2 to 1.5 wt. %, based on the weight of the resin solids of coating composition B.

As already mentioned, the process of the present invention allows to achieve both, the desired dark-color shade and the low heat development in sunlight, although coating compositions A and B and the clear coat composition are applied wet-on-wet-on-wet. The desired dark-color shade and the low heat development in sunlight can even be achieved when the wet-on-wet-on-wet coating process is carried out in the context of an industrial mass production coating process, i.e., in an industrial painting facility which allows only for short time intervals between the three paint application steps. The short time-intervals between the three paint application steps result from the fact that the substrates to be coated are moving along a continuously moving painting line.

#### DETAILED DESCRIPTION OF THE EMBODIMENTS

The term "dark-color multi-layer coating" is used in the description and the claims. It refers to multi-layer coatings exhibiting a brightness  $L^*$  (according to CIEL\*a\*b\*, DIN 6174), measured at an illumination angle of 45 degrees to the perpendicular and an observation angle of 45 degrees to the specular, of at most 10 units. Examples of such dark colors are corresponding dark-green, dark-blue, dark-red, dark-brown, dark-grey and black color shades and they include solid colors (single-tone colors) and special effect colors (colors characterized by color and/or brightness flop dependent on the angle of observation) like metallic and/or mica color shades.

The measurement of the brightness  $L^*$  at an illumination angle of 45 degrees to the perpendicular and an observation angle of 45 degrees to the specular is known to the person skilled in the art and can be carried out with commercial professional measuring instruments, for example, the instrument X-Rite MA 68 sold by the firm X-Rite Incorporated, Grandeville, Mich., USA.

The abbreviation "NIR" used in the description and the claims stands for "near infrared" or "near infrared radiation" and shall mean infrared radiation in the wavelength range of 780 to 2100 nm.

The term "NIR-opaque coating layer" is used in the description and the claims. It refers to a dried or cured pigmented coating layer with a film thickness at least as thick that underlying substrate surfaces (substrate surfaces located directly beneath the coating layer) with different NIR absorption are no longer discernible by NIR reflection measurement (no longer distinguishable from each other by NIR reflection measurement), i.e., at or above this minimum dry film thickness no difference can be determined when measuring the NIR reflection of the coating layer applied to such different substrate surfaces and dried or cured; or to put it into other words, the NIR reflection curve measured is then only determined by the NIR-opaque coating layer. In still other words, an NIR-opaque coating layer is characterized in that its dry film thickness corresponds to or exceeds said minimum film thickness, but may not fall below it. It goes without saying that this minimum film thickness depends on the pigmenta-

tion of the respective coating layer, i.e., it depends on the composition of the pigment content as well as on the pigment/resin solids weight ratio. In order to determine said minimum film thickness, the respective coating composition may be applied in a wedge shape onto a black and white chart and dried or cured. Black and white charts are typically used when determining black/white opacity of coating compositions (see, for example, ISO 6504-3:2006 (E), method B). NIR reflection measurement is known to the person skilled in the art and can be carried out making use of a conventional NIR spectrophotometer (measuring geometry 8°/d), for example, the instrument Lambda 19 sold by the firm Perkin-Elmer. NIR-opacity of an NIR-opaque coating layer can be the result of NIR absorption and/or NIR reflection and/or NIR scattering.

The term "film thickness" is used herein. It refers always to the dry film thickness of the respective dried or cured coating. Accordingly, any film thickness values indicated in the description and in the claims for coating layers refer in each case to dry film thicknesses.

The term "pigment content" is used herein. It means the sum of all the pigments contained in a coating composition without fillers (extenders, extender pigments). The term "pigments" is used here as in DIN 55944 and covers, in addition to special effect pigments, inorganic white, colored and black pigments and organic colored and black pigments. At the same time, therefore, DIN 55944 distinguishes between pigments and fillers.

The term "resin solids" is used herein. The resin solids of a coating composition consist of the solids contribution of the coating binders (binder solids) and the solids contribution of crosslinkers (crosslinker solids) contained in the coating composition.

The term "black/white opacity" is used herein. It refers to the dry film thickness of a pigmented coating composition wherein the contrast between the black and white fields of a black and white chart coated with the coating composition is no longer visually discernible (mean film thickness value determined on the basis of evaluation by 5 independent individuals). It goes without saying that this film thickness depends on the pigmentation of the respective coating layer, i.e., it depends on the composition of the pigment content as well as on the pigment/resin solids weight ratio. Following ISO 6504-3:2006 (E), method B, in order to determine said film thickness, the pigmented coating composition of which the black/white opacity is to be investigated may be applied in a wedge shape onto a black and white chart and dried or cured.

The term "coating layer A' exhibiting low NIR absorption" is used in the description and the claims. It shall mean an NIR-opaque coating layer A' which exhibits an NIR reflection of at least 48% over the entire NIR wavelength range of 780 to 2100 nm, i.e., at any wavelength within this NIR wavelength range. In case of the particular embodiment of the present invention, it shall mean an NIR-opaque coating layer A' which exhibits an NIR reflection of at least 55% over the entire NIR wavelength range of 780 to 2100 nm. The NIR reflection measurement can be carried out as explained above.

The term "coating layer B' exhibiting low NIR absorption" is used in the description and the claims. It shall mean a coating layer B' which would exhibit an NIR reflection of at least 33% over the entire NIR wavelength range of 780 to 2100 nm, if it were applied and dried or cured on an NIR-opaque coating layer pigmented exclusively with 100 to 1000 nm thick aluminum flake pigment with regard to the particular embodiment of the present invention, it shall mean a coating layer B' which would exhibit an NIR reflection of at

least 40% over the entire NIR wavelength range of 780 to 2100 nm, if it were applied and dried or cured on an NIR-opaque coating layer pigmented exclusively with 10 to 80 nm thick aluminum flake pigment. The person skilled in the art may, for example, produce test panels provided with a dried or cured coating layer applied from a coating composition pigmented exclusively with 100 to 1000 nm thick aluminum flake pigment or with 10 to 80 nm thick aluminum flake pigment, and may use said test panels as test substrates for coating with coating compositions to be tested for their NIR absorption. Once the coating layer applied from the coating composition to be tested has dried or cured, the NIR reflection of said coating layer can be measured. The NIR reflection measurement itself can be carried out as explained above. The method mentioned in this paragraph can be used by the skilled person when developing the pigmentation of a coating composition B.

In step (1) of the process of the present invention substrates are coated with an NIR-opaque coating layer A' exhibiting low NIR absorption. The substrates may comprise various materials including, for example, metals and plastics including metal parts, metal foils, plastic parts and plastic foils; parts may or may not comprise an interior. The substrates may be uncoated or provided with a precoating consisting of one or more coating layers. In particular, the uncoated or pre-coated substrates are substrates which exhibit considerable NIR absorption as a property of the substrate material itself and/or as a property of a precoating; this may be the case, for example, if the substrate material and/or at least one relevant coating layer of the precoating contain(s) a certain amount of pigments with strong NIR absorption such as carbon black, for example, 0.1 to 10 wt. % of carbon black. The substrate's include, in particular, vehicles which can be used for transporting people and/or goods as well as corresponding vehicle parts and accessories, wherein the term "vehicle" includes motorized and unmotorized vehicles including aircraft, water craft, rail vehicles and road vehicles. In particular, the substrates are road vehicles and road vehicle parts, more specifically car bodies, car body parts and car body fittings which have generally been precoated. Car bodies or car body parts made of metal generally comprise, for example, an electrodeposition primer and, optionally, a primer surfacer layer applied thereto whilst car body parts or car body fittings made of plastics material maybe provided with a plastics primer.

In an embodiment, the substrates comprise car bodies or car body metal parts provided with an electrodeposition primer, wherein the electrodeposition primer contains carbon black, for example, 0.5 to 4 wt. % of carbon black.

In a further embodiment, the substrates comprise car bodies or car body metal parts provided with an electrodeposition primer and a primer surfacer layer, wherein both the electrodeposition primer and the primer surfacer layer or only the primer surfacer layer contain(s) carbon black, for example, 0.5 to 4 wt. % of carbon black.

The invention is most useful in the context of coating substrates, such as, in particular car bodies or car body parts, in an industrial painting facility, in particular one which allows only for short time intervals between the three paint application steps (1), (2) and (4).

The NIR-opaque coating layer A' applied in step (1) of the process of the present invention is applied from a solvent-borne pigmented coating composition A.

Coating composition A comprises at least one component selected from the group consisting of (i) (a) >5 to 20 wt. % of cellulose ester binder and up to 10 wt. % of NAD binder or (b) 10 to 100 wt. % of NAD binder and up to 5 wt. % of cellulose ester binder, the wt. % in each case being based on the weight

of the binder solids of coating composition A, (ii) 0.2 to 1.5 wt. %, based on the weight of the resin solids of coating composition A, of sheet silicate, (iii) 0.5 to 2 wt. %, based on the weight of the resin solids of coating composition A, of fumed silica, (iv) 0.5 to 2.5 wt. %, based on the weight of the resin solids of coating composition A, of urea SCA and (v) 0.5 to 8 wt. %, based on the weight of the resin solids of coating composition A, of polyolefine wax.

In an embodiment, coating composition A comprises components (i) (a) and (v), namely >5 to 20 wt. % of cellulose ester binder and up to 10, preferably 0 wt. % of NAD binder, the wt. % in each case being based on the weight of the binder solids of coating composition A, and 0.5 to 8, preferably 3 to 8 wt. %, based on the weight of the resin solids of coating composition A, of polyolefine wax.

In another embodiment, coating composition A comprises components (i) (b) and (ii), or components (i) (b) and (iii), or components (i) (b), (ii) and (iii), namely 10 to 100, preferably 10 to 25 wt. % of NAD binder and up to 5 wt. % of cellulose ester binder, the wt. % in each case being based on the weight of the binder solids of coating composition A and 0.2 to 1.5, preferably 0.5 to 1 wt. %, based on the weight of the resin solids of coating composition A, of sheet silicate, or 10 to 100, preferably 10 to 25 wt. % of NAD binder and up to 5 wt. % of cellulose ester binder, the wt. % in each case being based on the weight of the binder solids of coating composition A and 0.5 to 2, preferably 0.5 to 1 wt. %, based on the weight of the resin solids of coating composition A, of fumed silica, or 10 to 100, preferably 10 to 25 wt. % of NAD binder and up to 5 wt. % of cellulose ester binder, the wt. % in each case being based on the weight of the binder solids of coating composition A and 0.2 to 1.5, preferably 0.5 to 1 wt. %, based on the weight of the resin solids of coating composition A, of sheet silicate and 0.5 to 2, preferably 0.5 to 1 wt. %, based on the weight of the resin solids of coating composition A, of fumed silica.

Coating composition A comprises resin solids. The resin solids consist of binder solids and crosslinker solids, for example, 60 to 85 wt. % of binder solids and, accordingly, 15 to 40 wt. % of crosslinker solids. The binder solids comprise one or more binder resins as are conventionally used in solvent-borne coating compositions and which are well-known to the skilled person. Examples of binders include (meth) acrylic copolymer binders, polyester binders, polyurethane binders and cellulose ester binders. (Meth)acryl is to be understood, both here and in the following, as acryl and/or methacryl. The binders may be soluble in organic solvent or they may take the form of an NAD in the solventborne coating system of coating composition A.

As already mentioned, coating composition A may contain cellulose ester binder as part of a component (i). The cellulose ester binders are, for example, cellulose acetopropionate or cellulose acetobutyrate, which are both sold commercially, for example, by the company Eastman, in various variants with different hydroxyl, acetyl and propionyl or butyryl contents. Cellulose acetobutyrate is preferred, particularly with high butyryl contents from 35 to 55 wt. % based on the weight of the cellulose ester.

As already mentioned, coating composition A may contain NAD binder as part of a component (i). The NAD binders maybe uncrosslinked or they may take the form of microgels, i.e. internally crosslinked polymer particles. Most preferred are (meth)acrylic copolymer NADs or microgels, which both are well known to the skilled person. Preparation of (meth) acrylic copolymer NADs is typically carried out by free-radical polymerization of olefinically unsaturated monomers including (meth)acrylic monomers in an organic solvent which is a solvent for the monomers but a non-solvent for the

(meth)acrylic copolymer formed in the course of the copolymerization. In case of the preparation of a (meth)acrylic copolymer microgel the olefinically unsaturated comonomers comprise a small amount of polyolefinically unsaturated monomers such as ethylene glycol di(meth)acrylate, hexene-diol di(meth)acrylate, allyl(meth)acrylate or divinylbenzene.

The binders making up the binder solids of coating composition A comprise at least one binder with functional groups capable of crosslinking with the melamine-formaldehyde resin crosslinker during thermal curing step (5) of the process of the present invention. Examples of such crosslinkable groups include in particular hydroxyl groups. It is preferred that the binder solids of coating composition A has a hydroxyl number of, for example, 20 to 150 mg KOH/g.

Furthermore the binder solids of coating composition A may comprise one or more paste resins (grinding resins; resins used for pigment grinding) or polymeric pigment wetting or dispersion aids.

The crosslinker solids of coating composition A consist 50 to 100 wt. % of melamine-formaldehyde resin crosslinker and, accordingly, 0 to 50 wt. % of further crosslinkers, for example, free or blocked polyisocyanate crosslinkers.

In an embodiment, the resin solids of coating composition A consist 60 to 85 wt. % of hydroxyl-functional binder solids and 15 to 40 wt. % of crosslinker solids, wherein the binder solids consist >5 to 20 wt. % of cellulose ester binder, up to 10 wt. % of (meth)acrylic copolymer NAD, in particular (meth)acrylic copolymer microgel, and 70 to <95 wt. % of one or more further binders, wherein the sum of the respective wt. % equals 100 wt. % in each case.

In a further embodiment, the resin solids of coating composition A consist 60 to 85 wt. % of hydroxyl-functional binder solids and 15 to 40 wt. % of crosslinker solids, wherein the binder solids consist up to 5 wt. % of cellulose ester binder, 10 to 100 wt. % of (meth)acrylic copolymer NAD, in particular (meth)acrylic copolymer microgel, and 0 to 90 wt. % of one or more further binders, wherein the sum of the respective wt. % equals 100 wt. % in each case.

Coating composition A comprises a pigment content consisting 90 to 100 wt. % of at least one aluminum flake pigment and 0 to 10 wt. % of at least one further pigment which is selected in such a way that NIR-opaque coating layer A' exhibits low NIR absorption, wherein the sum of the wt. % equals 100 wt. %. Generally, the pigment/resin solids ratio by weight of coating composition A is, for example, 0.1:1 to 1:1.

Generally, the at least one aluminum flake pigment comprises one or more 100 to 1000 nm thick aluminum flake pigments and optionally, one or more 10 to 80 nm thick aluminum flake pigments, wherein the proportion of the latter is such that it accounts for less than 90 wt. % of the pigment content of coating composition A. In an embodiment, the at least one aluminum flake pigment consists of one or more 100 to 1000 nm thick aluminum flake pigments.

In case of the particular embodiment, the at least one aluminum flake pigment is selected from 10 to 80 nm thick aluminum flake pigments. In this case, the pigment/resin solids ratio by weight of coating composition A is in the range of, for example, 0.05:1 to 0.5:1.

The 100 to 1000 nm thick aluminum flake pigments are special effect pigments and have a mean particle diameter of, for example, 5 to 50  $\mu\text{m}$ , preferably 5 to 35  $\mu\text{m}$ . The mean particle diameters may be inferred, for example, from the technical documents of manufacturers of such aluminum flake pigments. The aluminum flake pigments are, in particular, aluminum flake pigments of the leafing or preferably non-leaving type that are conventional in paint and coatings and are known to the person skilled in the art. The aluminum

flake pigments may be coated or uncoated. Coated types are, for example, coated with a silicon-oxygen network. Non-leaving aluminum flake pigments coated with a silicon-oxygen network and their production are also known, for example, from WO 99/57204, U.S. Pat. No. 5,332,767 and from A. Kiehl and K. Greiwe, Encapsulated aluminum pigments, Progress in Organic Coatings 37 (1999), pp. 179 to 183. The surface of the non-leaving aluminum flake pigments is provided with a coating of a silicon-oxygen network. The silicon-oxygen network can be connected to the surface of the non-leaving aluminum flake pigments via covalent bonds. The term "non-leaving aluminum flake pigments coated with a silicon-oxygen network" includes in accordance with the above explanations both non-leaving aluminum flake pigments with a coating of a purely inorganic silicon-oxygen network and non-leaving aluminum flake pigments with a coating of a silicon-oxygen network modified with corresponding organic groups or polymer-modified. Examples of commercially available non-leaving aluminum flake pigments coated with a silicon-oxygen network are the non-leaving aluminum flake pigments sold by Eckert under the name "STAPA IL Hydrolan®". Examples of commercially available non-leaving aluminum flake pigments having a fatty acid based boating are the non-leaving aluminum flake pigments sold by Eckert under the name "STAPA Metallux®" and those sold by Toyo Aluminum under the name "Alpaste TCR®".

The 10 to 80 nm, preferably 20 to 80 nm thick aluminum flake pigments are special effect pigments and have a mean particle diameter of, for example, 5 to 30  $\mu\text{m}$ , preferably 5 to 20  $\mu\text{m}$ . The mean particle diameters may be inferred, for example, from the technical documents of manufacturers of such aluminum flake pigments. The 10 to 80 nm thick aluminum flake pigments have an aspect ratio (the ratio of the flake diameter to the flake thickness) that is very high. The 10 to 80 nm thick aluminum flake pigments are produced, for example, by vacuum deposition or ultrathin grinding of special aluminum grits. The 10 to 80 nm thick aluminum flake pigments may be coated or uncoated. Coated types are, for example, (meth)acrylic resin coated or coated with a silicon-oxygen network. Examples of commercially available 10 to 80 nm thick aluminum flake pigments are those sold under the names Metalure®, Silvershine® and Hydroshine®, in each case by Eckart, Metasheen® by Ciba, Starbrite® by Silberline and Decomet® by Schlenk.

It is preferred that the pigment content of coating composition A consists exclusively of the at least one aluminum flake pigment. However, it may also comprise above 0 to 10 wt. % of at least one further pigment which is selected in such a way that NIR-opaque coating layer A' exhibits low NIR absorption. This means that, in case there is only one single further pigment, its wt. % proportion is selected within said range of above 0 to 10 wt. % such that NIR-opaque coating layer A' exhibits low NIR absorption; if the one single further pigment is a pigment with strong NIR absorption, the skilled person will select its wt. % proportion more at the lower end of said range of above 0 to 10 wt. %, whereas in case of one single further pigment with low NIR absorption the opposite is possible. In case there is a combination of two or more further pigments with different NIR absorption power the same principles apply and the proportion of each of the further pigments may accordingly be selected within the range of above 0 to 10 wt. %, i.e., taking into account the NIR absorption of each individual further pigment.

The person skilled in the art may easily determine the NIR absorption of a pigment, for example, by pigmenting a coating composition with the pigment in question and a 10 to 80

nm or a 100 to 1000 nm thick aluminum flake pigment in a pigment weight ratio of 10:90, i.e., without using other pigments, by applying and drying or curing the coating composition thus pigmented in an NIR-opaque film thickness, and by measuring the NIR reflection of the resultant coating layer over the entire wavelength range of 780 to 2100 nm. The NIR reflection can be measured as explained above for the measurement of the NIR reflection of an NIR-opaque coating layer.

The further pigment(s) that may be contained in coating composition A, in addition to the at least one aluminum flake pigment, may, for example, be other special effect pigments and/or pigments selected from white, colored and black pigments.

Examples of special effect pigments other than the at least one aluminum flake pigment include conventional pigments imparting to a coating a color and/or brightness flop dependent on the angle of observation, such as non-leaving metal pigments different from aluminum, interference pigments such as, for example, metal oxide-coated metal pigments, for example, iron oxide-coated aluminum, coated mica such as, for example, titanium dioxide-coated mica, iron oxide in flake form, liquid crystal pigments, coated aluminum oxide pigments, and coated silicon dioxide pigments. In case of the particular embodiment of the present invention, the foregoing list of examples may also include aluminum pigments other than 10 to 80 nm thick aluminum flake pigments, for example, 100 to 1009 nm thick aluminum flake pigments.

Examples of white, colored and black pigments are conventional inorganic or organic pigments known to the person skilled in the art, such as, for example, titanium dioxide, carbon black, iron oxide pigments, azo pigments, phthalocyanine pigments, quinacridone pigments, pyrrolopyrrole pigments, and perylene pigments.

It is preferred that coating composition A does not contain any carbon black.

With the exception of the at least one aluminum flake pigment as well as the possible additional special effect pigments, the other pigments that are optionally contained in the pigment content of coating composition A are generally ground. Grinding is generally performed until at least 70% of the maximum tinting strength achievable in the non-volatile system of coating composition A is achieved (non-volatile system of coating composition A means resin solids of coating composition A plus non-volatile additives of coating composition A). The determination of the maximum tinting strength is known to the person skilled in the art (compare, for example, DIN 53238). The grinding may be performed in conventional assemblies known to the person skilled in the art. Generally, the grinding takes place in a proportion of the binder or in a paste resin. The formulation is then completed with the remaining proportion of the binder or of the paste resin.

The at least one aluminum flake pigment and the optional additional special effect pigments are not ground, but are generally initially introduced in the form of a commercially available paste, optionally, combined with organic solvents and, optionally, polymeric pigment wetting or dispersion aids and/or other additives, and then mixed with the binder(s). Aluminum flake pigments and optional additional special effect pigments in powder form may first be processed with organic solvents and, optionally, polymeric pigment wetting or dispersion aids and/or other additives to yield a paste.

Coating composition A may contain one or more fillers in a total proportion of, for example, up to 20 wt. %, based on the resin solids. For the fillers the same principles apply as are valid for the at least one further pigment, i.e., they are selected

in such a way that NIR-opaque coating layer A' exhibits low NIR absorption. Examples are barium sulfate, kaolin, talcum, fumed silica, sheet silicate and any mixtures thereof. The fillers do not constitute part of the pigment content of coating composition A.

Coating composition A may contain sheet silicate. The sheet silicate may in particular be contained as a component (ii) in a proportion of 0.2 to 1.5 wt. %, based on the weight of the resin solids of coating composition A. Sheet silicate is known to the person skilled in the art and conventionally used in connection with coatings, for example, aluminum-magnesium, sodium-magnesium and sodium-magnesium-lithium silicates with a layered structure. Examples of such sheet silicates are sheet silicates of the bentonite, smectite, montmorillonite and hectorite type. Naturally occurring sheet silicates may be used, but synthetically manufactured sheet silicates are preferred. It may be convenient if the sheet silicates used are washed grades. Examples of commercially available sheet silicates which may be used in coating composition A are the Optigel® products (from Südchemie Moosburg, Germany), Bentone® (from Elementis) or Garamite® sheet silicates (from Southern Clay Products, US).

Coating composition A may contain fumed silica. The fumed silica may in particular be contained as a component (iii) in a proportion of 0.5 to 2 wt. %, based on the weight of the resin solids of coating composition A.

Coating composition A may contain conventional additives in a total quantity of, for example, 0.1 to 10 wt. %, relative to its resin solids content. Examples are wetting agents, adhesion promoters, catalysts, leveling agents, anti-cratering agents, rheology control agents and light stabilizers, for example, UV absorbers and/or HALS compounds (HALS, hindered amine light stabilizers).

Coating composition A may contain urea SCA. The urea SCA may in particular be contained as a component (iv) in a proportion of 0.5 to 2.5 wt. %, based on the weight of the resin solids of coating composition A. Urea SCAs are addition products of diisocyanates and/or polyisocyanates derived therefrom and mono- and/or polyamines. The addition products may be defined as low molecular weight compounds that can be defined by a molecular formula or oligomeric or polymeric addition products. Urea SCAs are preferably addition products of diisocyanates, preferably, aliphatic or cycloaliphatic diisocyanates, particularly, those having a symmetrical structure, and primary amines, preferably, primary monoamines. They are preferably solid, particularly preferably, crystalline urea compounds. A particularly preferred urea SCA compound is the adduct formed from 1 mole of hexane 1,6-diisocyanate and 2 mole of benzylamine. The urea SCA compounds may be prepared in the usual way by addition of amines having primary and/or secondary amino groups to polyisocyanates. The preparation takes place, for example, at temperatures from 20° C. to 80° C., for example, without solvents, in bulk, preferably, in an inert solvent or, particularly preferably, in the presence of binder or crosslinker that is inert under the reaction conditions, for example, an inert binder or crosslinker solution. If coating composition A contains more than one binder or more than one crosslinker, the preparation may take place, for example, in one of said binders or in one of said crosslinkers. The addition of the urea SCAs during the preparation of coating composition A takes place preferably in such a way that the urea SCAs are mixed with the constituents of coating composition A as a preparation, for example, as a dispersion in a solvent or, particularly preferably, as a dispersion in a part of the liquid binder or crosslinker. Further details about urea SCA compounds that may be used in coating composition A,

## 11

starting materials, processes and process parameters for the preparation of the urea SCA compounds and the incorporation thereof in coating compositions can be derived from U.S. Pat. Nos. 4,311,622, 4,677,028 and 4,851,294, to which express but not exclusive reference is made here.

Coating composition A may contain polyolefine wax as an additive. The polyolefine wax may in particular be contained as a component (v) in a proportion of 0.5 to 8 wt. %, based on the weight of the resin solids of coating composition A. Polyolefine waxes are based on homo- or copolymers of olefines like, in particular, ethylene. Such polyolefine waxes are commercially available from many suppliers as paint additives.

The overall solids content of coating composition A is in the range of 15 to 40 wt. %, based on the total composition. Accordingly, the portion of volatiles (volatile materials) is 60 to 85 wt. %. The volatiles comprise the organic solvent carrier and possible volatile additives. Examples of organic solvents which can be used in coating composition A include alcohols, for example, propanol, butanol, hexanol; glycol ethers, for example, diethylene glycol di-C1-C6-alkyl ether, dipropylene glycol di-C1-C6-alkyl ether, ethoxypropanol, ethylene glycol monobutyl ether; glycol esters, for example, ethylene glycol monobutyl ether acetate; esters, for example, butyl acetate, amyl acetate; glycols, for example, ethylene glycol and/or propylene glycol, and the di- or trimers thereof; ketones, for example, methyl ethyl ketone, acetone, cyclohexanone; aromatic or aliphatic hydrocarbons, for example, toluene, xylene or linear or branched aliphatic C6-C12 hydrocarbons.

In step (2) of the process of the present invention coating layer B' is applied from a solventborne pigmented coating composition B.

Coating composition B comprises at least one component selected from the group consisting of (i') (a) >5 to 20 wt. % of cellulose ester binder and up to 10 wt. % of NAD binder or (b) 10 to 100 wt. % of NAD binder and up to 5 wt. % of cellulose ester binder, the wt. % in each case being based on the weight of the binder solids of coating composition B, (ii') 0.2 to 1.5 wt. %, based on the weight of the resin solids of coating composition B, of sheet silicate, (iii') 0.5 to 2 wt. %, based on the weight of the resin solids of coating composition B, of fumed silica, (iv') 0.5 to 2.5 wt. %, based on the weight of the resin solids of coating composition B, of urea SCA and (v') 0.5 to 8 wt. %, based on the weight of the resin solids of coating composition B, of polyolefine wax.

In an embodiment, coating composition B comprises components (i') (a) and (v'), namely >5 to 20 wt. % of cellulose ester binder and up to 10, preferably 0 wt. % of NAD binder, the wt. % in each case being based on the weight of the binder solids of coating composition B, and 0.5 to 8, preferably 3 to 8 wt. %, based on the weight of the resin solids of coating composition B, of polyolefine wax.

In another embodiment, coating composition B comprises components (i') (b) and (ii'), or components (i') (b) and (iii'), or components (i') (b), (ii') and namely 10 to 100, preferably 10 to 25 wt. % of NAD binder and up to 5 wt. % of cellulose ester binder, the wt. % in each case being based on the weight of the binder solids of coating composition B and 0.2 to 1.5, preferably 0.5 to 1 wt. %, based on the weight of the resin solids of coating composition B, of sheet silicate, or 10 to 100, preferably 10 to 25 wt. % of NAD binder and up to 5 wt. % of cellulose ester binder, the wt. % in each case being based on the weight of the binder solids of coating composition B and 0.5 to 2, preferably 0.5 to 1 wt. %, based on the weight of the resin solids of coating composition B, of fumed silica, or 10 to 100, preferably 10 to 25 wt. % of NAD binder and up to 5 wt. % of cellulose ester binder, the wt. % in each case being based

## 12

on the weight of the binder solids of coating composition B and 0.2 to 1.5, preferably 0.5 to 1 wt. %, based on the weight of the resin solids of coating composition B, of sheet silicate and 0.5 to 2, preferably 0.5 to 1 wt. %, based on the weight of the resin solids of coating composition B, of fumed silica.

Coating composition B comprises resin solids. The resin solids consist of binder solids and crosslinker solids, for example, 60 to 85 wt. % of binder solids and, accordingly, 15 to 40 wt. % of crosslinker solids. The binder solids comprise 10 one or more binder resins as are conventionally used in solvent-borne coating compositions and which are well-known to the skilled person. Examples of binders include (meth) acrylic copolymer binders, polyester binders, polyurethane binders and cellulose ester binders. The binders may be 15 soluble in organic solvent or they may take the form of an NAD in the solventborne coating system of coating composition B.

As already mentioned, coating composition B may contain cellulose ester binder as part of a component (i'). With regard 20 to the cellulose ester binder the same is true as has been mentioned above in connection with coating composition A. Therefore, to avoid unnecessary repetitions reference is made to the corresponding paragraph above.

As already mentioned, coating composition B may contain 25 NAD binder as part of a component (i'). With regard to the NAD binder the same is true as has been mentioned above in connection with coating composition A. Therefore, to avoid unnecessary repetitions reference is made to the corresponding paragraphs above.

The binders making up the binder solids of coating composition B comprise at least one binder with functional groups capable of crosslinking with the melamine-formaldehyde resin crosslinker during thermal curing step (5) of the process of the present invention. Examples of such crosslinkable groups include in particular hydroxyl groups. It is preferred that the binder solids of coating composition B has a hydroxyl number of, for example, 20 to 150 mg KOH/g.

Furthermore the binder solids of coating composition B may comprise one or more paste resins or polymeric pigment 40 wetting or dispersion aids.

The crosslinker solids of coating composition B consist 50 to 100 wt. % of melamine-formaldehyde resin crosslinker and, accordingly, 0 to 50 wt. % of further crosslinkers, for example, free or blocked polyisocyanates crosslinkers.

In an embodiment, the resin solids of coating composition B consist 60 to 85 wt. % of hydroxyl-functional binder solids and 15 to 40 wt. % of crosslinker solids, wherein the binder solids consist >5 to 20 wt. % of cellulose ester binder, up to 10 wt. % of (meth)acrylic copolymer NAD, in particular (meth) acrylic copolymer microgel, and 70 to <95 wt. % of one or more further binders, wherein the sum of the respective wt. % equals 100 wt. % in each case.

In a further embodiment, the resin solids of coating composition B consist 60 to 85 wt. % of hydroxyl-functional 55 binder solids and 15 to 40 wt. % of crosslinker solids, wherein the binder solids consist up to 5 wt. % of cellulose ester binder, 10 to 100 wt. % of (meth)acrylic copolymer NAD, in particular (meth)acrylic copolymer microgel, and 0 to 90 wt. % of one or more further binders, wherein the sum of the respective wt. % equals 100 wt. % in each case.

Coating composition B'comprises a pigment content consisting 50 to 100 wt. % of at least one black pigment with low NIR absorption and 0 to 50 wt % of at least one further pigment which is selected in such a way that coating layer B' 65 exhibits low NIR absorption and that the multi-layer coating produced by the process of the present invention exhibits a brightness L\* (according to CIEL\*a\*b\*, DIN 6174), mea-

sured at an illumination angle of 45 degrees to the perpendicular and an observation angle of 45 degrees to the specular, of at most 10 units, wherein the sum of the wt. % equals 100 wt. %. The pigment/resin solids ratio by weight of coating composition B is, for example, 0.1:1 to 1:1.

A black pigment with low NIR absorption is one which, when pigmenting a coating composition with the respective black pigment and a 100 to 1000 nm thick aluminum flake pigment in a pigment weight ratio of 10:90 and without using other pigments, results in the NIR reflection of a dried or cured coating layer applied from the coating composition in an NIR-opaque film thickness being at least 33% over the entire wavelength range of 780 to 2100 nm. The NIR reflection can be measured as explained above for the measurement of the NIR reflection of an NIR-opaque coating layer. Preferred examples of black pigments with low NIR absorption are iron oxide black pigments, mixed metal/iron oxide black pigments, for example, of the inverse spinel type, and, in particular, perylene black pigments. Examples of commercially available perylene black pigments are Paliogen® Black L 0084 and Paliogen® Black L 0086 from BASF.

The pigment content of coating composition B may consist exclusively of the at least one black pigment with low NIR absorption or it may also comprise above 0 to 50 wt. % of at least one further pigment which is selected in such a way that coating layer B' exhibits low NIR absorption and that the dark-color multi-layer coating produced by the process of the present invention exhibits a brightness L\* (according to CIEL\*a\*b\*, DIN 6174), measured at an illumination angle of 45 degrees to the perpendicular and an observation angle of 45 degrees to the specular, of at most 10 units. In other words, the selection of the at least one further pigment is performed in a manner meeting two conditions, namely condition (i) relating to the low NIR absorption of coating layer B and, simultaneously, condition (ii) relating to the brightness L\* of the dark-color multi-layer coating of at most 10 units.

This means with regard to condition (i): In case there is only one single further pigment its wt. % proportion is selected within said range of above 0 to 50 wt. % such that coating layer B' exhibits low NIR absorption; if the one single further pigment is a pigment with strong NIR absorption, the skilled person will select its wt. % proportion more at the lower end of said wt. % range, whereas in case of one single further pigment with low NIR absorption the opposite is possible. In case there is a combination of two or more further pigments with different NIR absorption power the same principles apply and the proportion of each of the further pigments may accordingly be selected within the range of above 0 to 50 wt. %, i.e., taking into account the NIR absorption of each individual further pigment.

At the same time this means with regard to condition (ii): In case there is only one single further pigment its wt. % proportion is selected within said range of above 0 to 50 wt. % such that the dark-color multi-layer coating exhibits a brightness L\* (according to CIEL\*a\*b\*, DIN 6174), measured at an illumination angle of 45 degrees to the perpendicular and an observation angle of 45 degrees to the specular, of at most 10 units; if the one single further pigment has a light color, the skilled person will not select its wt. % proportion at the upper end of said wt. % range, whereas in case of one single further pigment with a dark color this may be possible. In case there is a combination of two or more further pigments with not only different color but also different brightness the same principles apply and the proportion of each of the further pigments may accordingly be selected within the range of above 0 to 50 wt. %, i.e., taking into account the brightness of each individual further pigment.

The further pigment(s) that may optionally be contained in coating composition B, in addition to the at least one black pigment with low NIR absorption may, for example, be special effect pigments and/or pigments selected from white, colored and other black pigments (black pigments different from the black pigments with low NIR absorption).

Examples of special effect pigments that may be contained in coating composition B comprise the aluminum flake pigments as are contained in coating composition A and the special effect pigments that have been previously mentioned as examples of special effect pigments that may be contained in coating composition A in addition to the at least one aluminum flake pigment.

Examples of white, colored and other black pigments are conventional inorganic or organic pigments known to the person skilled in the art, such as, for example, titanium dioxide, carbon black, iron oxide pigments different from iron oxide black pigments, azo pigments, phthalocyanine pigments, quinacridone pigments, pyrrolopyrrole pigments, and perylene pigments different from perylene black pigments.

It is preferred that coating composition B does not contain any carbon black.

With the exception of the possible special effect pigments, the black pigment(s) with low NIR absorption and the possible further pigments are generally ground. Grinding is generally performed until at least 70% of the maximum tinting strength achievable in the non-volatile system of coating composition B is achieved (non-volatile system of coating composition B means resin solids of coating composition B plus non-volatile additives of coating composition B). The grinding may be performed in conventional assemblies known to the person skilled in the art. Generally, the grinding takes place in a proportion of the binder or in specific paste resins. The formulation is then completed with the remaining proportion of the binder or of the paste resin.

The possible special effect pigments are not ground, but are generally initially introduced in the form of a commercially available paste, optionally, combined with organic solvents and, optionally, polymeric pigment wetting or dispersion aids and/or other additives, and then mixed with the binder(s). Special effect pigments in powder form may first be processed with organic solvents and, optionally, polymeric pigment wetting or dispersion aids and/or other additives to yield a paste.

Coating composition B may contain one or more fillers in a total proportion of, for example, up to 20 wt. %, based on the resin solids. For the fillers the same principles apply as are valid for the at least one further pigment, i.e., they are selected in such a way that NIR-opaque coating layer B' exhibits low NIR absorption. Examples are barium sulfate, kaolin, talcum, fumed silica, sheet silicate and any mixtures thereof. The fillers do not constitute part of the pigment content of coating composition B.

Coating composition B may contain sheet silicate. The sheet silicate may in particular be contained as a component (ii') in a proportion of 0.2 to 1.5 wt. %, based on the weight of the resin solids of coating composition B. Examples of suitable sheet silicates are the same as those mentioned above in connection with coating composition A.

Coating composition B may contain fumed silica. The fumed silica may in particular be contained as a component (iii') in a proportion of 0.5 to 2 wt. %, based on the weight of the resin solids of coating composition B.

Coating composition B may contain conventional additives in a total quantity of, for example, 0.1 to 10 wt. %, relative to its resin solids content. Examples are wetting agents, adhesion promoters, catalysts, leveling agents, anti-

## 15

cratering agents, rheology control agents and light stabilizers, for example, UV absorbers and/or HALS compounds (HALS, hindered amine light stabilizers).

Coating composition B may contain urea SCA. The urea SCA may in particular be contained as a component (iv') in a proportion of 0.5 to 2.5 wt. %, based on the weight of the resin solids of coating composition B. With regard to the urea SCA the same is true as has been mentioned above in connection with coating composition A. Therefore, to avoid unnecessary repetitions reference is made to the corresponding paragraph above.

Coating composition B may contain polyolefine wax as an additive. The polyolefine wax may in particular be contained as a component (v') in a proportion of 0.5 to 8 wt. %, based on the weight of the resin solids of coating composition B.

The overall solids content of coating composition B is in the range of 15 to 40 wt. %, based on the total composition. Accordingly, the proportion of volatiles is 60 to 85 wt. %. The volatiles comprise the organic solvent carrier and possible volatile additives. Examples of organic solvents which can be used in coating composition B are the same as those mentioned above in connection with coating composition A.

The multi-layer coating process of the present invention comprises the successive steps (1) to (5) in the course of the process, coating layers A', B' and the clear coat layer are applied wet-on-wet-on-wet and simultaneously cured.

In step (1) of the process of the present invention coating composition A is applied in a film thickness so as to form an NIR-opaque coating layer A' exhibiting low NIR absorption. Generally the film thickness of coating layer A' will then also correspond to at least black/white opacity or be even higher. Not least for cost reasons NIR-opaque coating layer A' is not applied unnecessarily thick. Generally the film thickness of coating layer A' is in the range of, for example, 7 to 30  $\mu\text{m}$ , preferably 9 to 20  $\mu\text{m}$ . In case of the particular embodiment of the present invention, the film thickness of coating layer A' is generally lower and is in the range of, for example, 2 to 20  $\mu\text{m}$ , preferably 4 to 10  $\mu\text{m}$ . Application may be performed by any coating application method, in particular, spray coating including, for example, pneumatic and/or bell application. The spray application may be electrostatically assisted.

In step (2) of the process according to the invention coating composition B is applied onto the substrate provided with coating layer A'.

Coating composition B may be applied in a relatively thin film thickness to form a transparent coating layer B'; generally, the film thickness of a transparent coating layer B' is in the range of, for example, 4 to 20  $\mu\text{m}$ . It is preferred however, that coating composition B is applied sufficiently thick so as to form a visually opaque coating layer B'; then its film thickness corresponds to or exceeds black/white opacity. The dry film thickness of a visually opaque coating layer B' is higher than that of a transparent coating layer B' and is generally in the range of for example, 8 to 30  $\mu\text{m}$ .

As already mentioned, coating layer B' may be transparent, and in this case the color shade of the dark-color multi-layer coating is determined by the contributions of both coating layers A' and B', although in general coating layer B' makes the main contribution to the color shade of the dark-color multi-layer coating. If coating layer B' is a visually opaque coating layer, it is the coating layer which determines the color shade of the dark-color multi-layer coating.

In the practice of the present invention, coating composition B can be applied over coating layer A' before the latter is dry. There may be no substantial evaporation of the volatiles from coating layer A' during the time between the completion of the application of coating composition A and the start of the

## 16

application of coating composition B. In an embodiment, coating composition B can even be applied to coating layer A' in such a manner that at least 50 wt. % of the volatiles of coating composition A are still present in coating layer A' when coating composition B is applied.

Coating composition B can be applied within, for example, 10 to 600 seconds, preferably within 1 to 7 minutes or even 1 to 4 minutes, of the application of coating composition A even under ambient conditions. Ambient conditions mean the environmental conditions in a typical industrial painting facility, for example, a temperature in the range of 15°C. to 35°C., in particular 18°C. to 28°C., a relative humidity in the range of 5 to 90%, in particular 50 to 70%, and, for a continuously moving painting line, a line speed in the range of 2 to 11 meters/minute. It is desirable to omit process steps that are not required, and thereby improve efficiency and reduce costs associated with such steps. It is thus an advantage that a forced or flash drying step between the application of coating compositions A and B is not required. As the person skilled in the art knows, forced or flash drying requires utilizing equipment such as blowers and/or heaters to remove volatiles at a faster rate than would occur under ambient conditions, or with ambient (unforced) air flow such as, for example, the normal airflow resulting from the movement of a substrate through space on a continuously moving painting line.

Application of coating composition B may be performed by any coating application method, in particular, spray coating including, for example, pneumatic and/or bell application. The spray application maybe electrostatically assisted. Coating composition B can be applied at essentially the same temperature, humidity, and airflow conditions, i.e., under the same or similar spraybooth conditions, as used to apply coating composition A.

In step (3) of the process of the present invention the substrate provided with both coating layers A' and B' is subjected to a drying step to evaporate volatiles from coating layers A' and B' and set, but not initiate curing or crosslinking of, the coating layers A' and B' on the substrate. By set, it is meant that coating layers A' and B' are dried sufficiently that they are not disturbed or marred (waved or rippled) by air currents that may blow past the surface. In a preferred embodiment the volatiles are removed until a solids content of coating layers A' and B' of >90 wt. % is reached. The drying step can be conducted at an air temperature of, for example, 20 to 40°C. The evaporation of volatiles from the coating layers A' and B' can be carried out in open air, but is preferably carried out in a drying chamber in which air is circulated at low velocity to minimize airborne particle contamination. A typical drying chamber has blowers or fans positioned at the top and sides of the chamber so that the circulated air is directed in a manner that is substantially perpendicular to the surface of the substrate. The substrate can be moved through the drying chamber in an assembly-line manner at a rate that permits the evaporation of volatiles from the applied coating layers A' and B' as discussed above. The rate at which the substrate is moved through the drying chamber depends in part upon the length and configuration of the chamber. The drying step can take from, for example, 30 seconds to 10 minutes, in particular 2 to 5 minutes, as in an industrial mass-production coating process.

In step (4) of the process of the present invention a clear coat is applied by the wet-on-wet-on-wet paint application method, i.e., the clear coat is applied onto the still uncured coating layer B' (and the still uncured coating layer A' located beneath the still uncured coating layer B'). Generally such outer clear coat does not or essentially not contribute to the color shade of the dark-color multi-layer coating.

All known solventborne clear coats are in principle suitable as clear coat. Usable clear coats are here both solventborne one-component (1 pack) or two-component (2 pack) clear coats.

Clear coat application may be performed in a film thickness of, for example, 20 to 60  $\mu\text{m}$  by any suitable coating application method, in particular, spray coating. The clear coat layer so applied may be subject to a short flash-off period of, for example, 2 to 10 minutes at ambient temperatures in the range of, for example, 20 to 40°C.

As already mentioned, the process of the present invention comprises a final step (5) of thermal curing the coating layers applied in process steps (1), (2), and (4). The curing of the three coating layers (coating layers A', B' and the clear coat layer) is performed simultaneously as a joint thermal curing step (heat curing step), for example, a single bake. The term "curing" used in the present description and the claims shall mean "crosslinking by formation of chemical bonds". Joint thermal curing of the three coating layers is performed by application of heat, for example, baking at an object temperature in the range of, for example, 120 to 180°C.

## EXAMPLES

Unless otherwise noted, all components of the following examples are believed to be available from the Aldrich Chemical Company, Milwaukee, Wis. The following other components were used in the examples.

CYMEL® 1168, melamine formaldehyde resin available from Cytec Industries Inc. West Patterson, N.J.

High solids acrylic polymer, as disclosed in US 2008/0131607 A1, page 8, Acrylic Polymer #4.

Dispersant #1, as disclosed in U.S. Pat. No. 6,472,463 B1, Example 6.

Dispersant #2, as disclosed in U.S. Pat. No. 6,472,463 B1, Example 8.

Microgel resin, as disclosed in US 2008/0131607 A1, example on pages 8-9.

Nacure® XP 221, sulphonic acid catalyst available from King Industries Norwalk, Conn.

PALIOGEN® BLACK L 0086, perylene black pigment available from BASF, Germany.

RAVEN 5000®, carbon black pigment available from Columbia Chemical Co., Marietta, Ga.

GARAMITE 2578®, sheet silicate available from Southern Clay Products, Gonzales, Tex.

ALPATE® 7670, aluminum pigment available from Toyal Europe, distributed by Krahn Chemie, Germany.

### Preparation of a Carbon Black Pigment Dispersion:

The following pigment slurry was prepared with 50.8 g (grams) of butyl acetate, 26.4 g of dispersant #1 and 4.8 g of dispersant #2. The above components were mixed together, 18 g of RAVEN 5000® was added and the resulting slurry was pre-dispersed using a Cowles blade. The mixture was then ground in a horizontal beadmill until the desired particle size of less than 0.5  $\mu\text{m}$  was achieved.

### Preparation of a Perylene Black Pigment Dispersion:

The following pigment slurry was prepared with 48.6 g of butyl acetate, 25.3 g of dispersant #1 and 4.6 g of dispersant #2. These components were mixed together, 21.5 g of PALIOGEN® BLACK L 0086 was added and the resulting slurry was pre-dispersed using a Cowles blade. The mixture was then ground in a horizontal beadmill until the desired particle size of less than 0.5  $\mu\text{m}$  was achieved.

### Preparation of a Rheology Base:

54.4 pbw (parts by weight) of butyl propionate was added to a mixing mill under a nitrogen atmosphere. 7.6 pbw of

GARAMITE 02578 was added with stirring. After stirring for 20 minutes, 38.0 pbw of high solids acrylic polymer was added. After stirring for 60 minutes the mixture was passed through the mill three times using zirconia media (0.8-1.0 mm).

### Preparation of a Solventborne Carbon Black Coating Composition:

A solventborne carbon black coating composition was prepared by mixing together the following constituents under constant agitation in the order stated: 34.2 pbw of high solids acrylic polymer, 11.6 pbw of carbon black pigment dispersion, 13.7 pbw of CYMEL® 1168, 9.4 pbw of rheology base, 12.4 pbw of microgel resin, 0.9 pbw of Nacure® XP 221, 6.3 pbw of isopropanol and 11.5 pbw of Solvesso® 100. The flow time of the coating composition was adjusted to 22 seconds with Ford cup No. 4 (4 mm), using 17.6 pbw of Solvesso® 100.

### Preparation of a Solventborne Perylene Black Coating Composition 1:

A solventborne perylene black coating composition was prepared by mixing together the following constituents under constant agitation in the order stated: 31.8 pbw of high solids acrylic polymer, 17.7 pbw of perylene black pigment dispersion, 12.8 pbw of CYMEL® 1168, 8.7 pbw of rheology base, 11.6 pbw of microgel resin, 0.9 pbw of Nacure® XP 221, 5.9 pbw of isopropanol and 10.6 pbw of Solvesso® 100. The flow time of the coating composition was adjusted to 22 seconds with Ford cup No. 4 (4 mm), using 17.6 pbw of Solvesso® 100.

### Preparation of a Comparative Solventborne Perylene Black Coating Composition 2:

This example shows the preparation of a solventborne perylene black coating composition without the addition of sheet silicate.

A solventborne perylene black coating composition was prepared by mixing together the following constituents under constant agitation in the order stated: 34.8 pbw of high solids acrylic polymer, 19.4 pbw of perylene black pigment dispersion, 14.0 pbw of CYMEL® 1168, 12.7 pbw of microgel resin, 1.0 pbw of Nacure® XP 221, 6.5 pbw of isopropanol and 11.6 pbw of Solvesso® 100. The flow time of the coating composition was adjusted to 22 seconds with Ford cup No. 4 (4 mm), using 1.0 pbw of Solvesso® 100.

### Preparation of a Comparative Solventborne Perylene Black Coating Composition 3:

This example shows the preparation of a solventborne perylene black coating composition without the addition of microgel.

The preparation of the solventborne perylene black coating composition 1 was repeated with the difference that the entire portion of the microgel resin was replaced by the high solids acrylic polymer. This replacement was performed according to an 1:1 replacement of binder solids. The flow time of the coating composition was adjusted to 22 seconds with Ford cup No. 4 (4 mm), using 14.0 pbw of Solvesso® 100.

### Preparation of a Solventborne Silver Coating Composition 1:

A solventborne silver coating composition was prepared by mixing together the following constituents under constant agitation in the order stated: 25.5 pbw of high solids acrylic polymer, 10.5 pbw of ALPATE® 7670, 12.7 pbw of CYMEL® 1168, 13.7 pbw of rheology base, 16.6 pbw of microgel resin, 4.7 pbw of butyl acetate, 0.8 pbw of Nacure® XP 221, 7.3 pbw of isopropanol and 8.2 pbw of Solvesso® 100. The flow time of the coating composition was adjusted to 22 seconds with Ford cup No. 4 (4 mm), using 19.0 pbw of Solvesso® 100.

## Preparation of a Comparative Solventborne Silver Coating Composition 2:

This example shows the preparation of a solventborne silver coating composition without the addition of sheet silicate.

A solventborne silver coating composition was prepared by mixing together the following constituents under constant agitation in the order stated: 29.5 pbw of high solids acrylic polymer, 12.2 pbw of ALPATE® 7670, 14.7 pbw of CYMEL® 1168, 19.2 pbw of microgel resin, 5.6 pbw of butyl acetate, 0.8 pbw of Nacure® XP 221, 8.5 pbw of isopropanol and 9.5 pbw of Solvesso® 100. The flow time of the coating composition was adjusted to 22 seconds with Ford cup No. 4 (4 mm) using 1.0 pbw of Solvesso® 100.

## Preparation of a Comparative Solventborne Silver Coating Composition 3:

This example shows the preparation of a solventborne silver coating composition without the addition of microgel.

The preparation of the solventborne silver coating composition 1 was repeated with the difference that the entire portion of the microgel resin was replaced by the high solids acrylic polymer. This replacement was performed according to an 1:1 replacement of binder solids. The flow time of the coating composition was adjusted to 22 seconds with Ford cup No. 4 (4 mm), using 18.0 pbw of Solvesso® 100.

## Solventborne Clear Coat Composition:

The clear coat composition used for the examples was a collision baking clear, commercially available from DuPont Performance Coatings (Standox), Christbusch 25, D-42285 Wuppertal, Germany, prepared by mixing STANDOCRYL® 2K-HS Clearcoat, 020-82497, with STANDOX® 2K-HS Hardener, 020-82403, in a 2:1 volume ratio.

## Application of Solventborne Coating Compositions and Clear Coat:

10.5 cm×30 cm, 1 mm thick steel test panels were processed and prepared with standard automotive pre-treatment, and dried and cured layers of grey electrocoat and midgrey primer.

The test panels were coated by spray-applying the solventborne silver coating compositions onto the surface of the midgrey primer. The solventborne silver coating compositions were spray-applied in 12 µm dry layer thickness and dried for 2 minutes at 20° C. Then the solventborne black coating compositions were spray-applied in 10 µm dry layer thickness and dried for 5 minutes at 20° C. Finally the clear coat was spray-applied in 40 µm dry layer thickness and dried for 5 minutes at 20° C. The test panels were then put in an oven and bake cured for 20 minutes at 145° C. (object temperature).

The test panels so provided with a black multi-layer coating different from each other were tested as follows:

A rectangular, open wooden box (dimensions inside 9.5 cm×29.4 cm, dimensions outside 12.6 cm×31.9 cm, height inside 5 cm and height outside 6.5 cm) was provided with a digital thermometer inside. To this end, the temperature sensor was fixed on a copper panel (8.5 cm×25.3 cm, thickness 1 mm) at the bottom inside the box. The box was closed by using one of the 10 cm×30 cm black coated test panels as a lid with the black coated surface turned outside. Then the box was put on a table and illuminated from above with a halogen lamp (Osram, No. 64575, 1000 W) over 35 min (simulation of heating up in sunlight). The distance between the black coated test panel surface and the light source was 35 cm and the temperature in the test room was 23° C. The temperature increase  $\Delta T$  within the box was measured.

The test panels were also visually assessed concerning color and occurrence of any unwanted sparkle effect (ok, no

unwanted sparkling; nok, not ok, occurrence of unwanted sparkling spots in the black coating).

Table 1 shows the results.

TABLE 1

|    | Multi-layer coating on the test panel:                                                             | AT (° C.) | Visual test |
|----|----------------------------------------------------------------------------------------------------|-----------|-------------|
| 10 | Solventborne silver coating 1 + carbon black coating + clear coat (comparative example)            | 20.8      | ok          |
|    | Solventborne silver coating 1 + perylene black coating 1 + clear coat (according to the invention) | 13.3      | ok          |
|    | Solventborne silver coating 1 + perylene black coating 2 + clear coat (comparative example)        | 13.1      | nok         |
| 15 | Solventborne silver coating 1 + perylene black coating 3 + clear coat (comparative example)        | 12.7      | nok         |
|    | Solventborne silver coating 2 + perylene black coating 1 + clear coat (comparative example)        | 11.9      | nok         |
|    | Solventborne silver coating 3 + perylene black coating 1 + clear coat (comparative example)        | 13.2      | nok         |

What is claimed is:

1. A process for the production of a dark-color multi-layer coating, comprising the successive steps:

- (1) applying an NIR-opaque coating layer A' from a solventborne pigmented coating composition A to a substrate,
- (2) applying a coating layer B' from a solventborne pigmented coating composition B onto the substrate provided with coating layer A',
- (3) subjecting the coated substrate obtained in step (2) to a drying step,
- (4) applying a clear coat layer from a clear coat composition onto the coated substrate obtained in step (3), and
- (5) thermally curing the coating layers applied in steps (1), (2), and (4) simultaneously;

wherein both coating compositions A and B comprise resin solids consisting of binder solids plus crosslinker solids comprising melamine-formaldehyde resin crosslinker, wherein coating composition A comprises at least one component selected from the group consisting of (i) (a) >5 to 20 wt. % of cellulose ester binder and up to 10 wt. % of NAD binder or (b) 10 to 100 wt. % of NAD binder and up to 5 wt. % of cellulose ester binder, the wt. % in each case being based on the weight of the binder solids of coating composition A, (ii) 0.2 to 1.5 wt. %, based on the weight of the resin solids of coating composition A, of sheet silicate, (iii) 0.5 to 2 wt. %, based on the weight of the resin solids of coating composition A, of fumed silica, (iv) 0.5 to 2.5 wt. %, based on the weight of the resin solids of coating composition A, of urea SCA and (v) 0.5 to 8 wt. %, based on the weight of the resin solids of coating composition A, of polyolefine wax, wherein coating composition B comprises at least one component selected from the group consisting of (i') (a) >5 to 20 wt. % of cellulose ester binder and up to 10 wt. % of NAD binder or (b) 10 to 100 wt. % of NAD binder and up to 5 wt. % of cellulose ester binder, the wt. % in each case being based on the weight of the binder solids of coating composition B, (ii') 0.2 to 1.5 wt. %, based on the weight of the resin solids of coating composition B, of sheet silicate, (iii') 0.5 to 2 wt. %, based on the weight of the resin solids of coating composition B, of fumed silica, (iv') 0.5 to 2.5 wt. %, based on the weight of the resin solids of coating composition B, of urea SCA and (v') 0.5 to 8 wt. %, based on the weight of the resin solids of coating composition B, of polyolefine wax,

**21**

wherein the pigment content of coating composition A consists 90 to 100 wt. % of at least one aluminum flake pigment and 0 to 10 wt. % of at least one further pigment, which is selected in such a way that NIR-opaque coating layer A' exhibits an NIR reflection of at least 48% over the entire NIR wavelength range of 780 to 2100 nm, wherein the pigment content of coating composition B consists 50 to 100 wt. % of at least one black pigment with low MR absorption and 0 to 50 wt. % of at least one further pigment, which is selected in such a way that coating layer B' exhibits an NIR reflection of at least 33% over the entire NIR wavelength range of 780 to 2100 nm, if it were applied and dried or cured on an NIR-opaque coating layer pigmented exclusively with 100 to 1000 nm thick aluminum flake pigment, and that the dark-color multi-layer coating exhibits a brightness L\* (according to CIEL\*a\*b\*, DIN 6174), measured at an illumination angle of 45 degrees to the perpendicular and an observation angle of 45 degrees to the specular, of at most 10 units.

2. The process of claim 1, wherein the at least one aluminum flake pigment consists of one or more 100 to 1000 nm thick aluminum flake pigments.
3. The process of claim 1, wherein the at least one aluminum flake pigment consists of one or more 10 to 80 nm thick aluminum flake pigments.
4. The process of claim 1, wherein coating composition A does not contain any carbon black.

**22**

5. The process of claim 1, wherein coating composition A comprises components (i) (a) and (v).

6. The process of claim 1, wherein coating composition A comprises components (i) (b) and (ii), or components (i) (b) and (iii), or components (i) (b), (ii) and (iii).

7. The process of claim 1, wherein the at least one black pigment with low NIR absorption is selected from the group consisting of iron oxide black pigments, mixed metal/iron oxide black pigments and perylene black pigments.

10 8. The process of claim 1, wherein coating composition B does not contain any carbon black.

9. The process of claim 1, wherein coating composition B comprises components (i') (a) and (v').

10 10. The process of claim 1, wherein coating composition B comprises components (i') (b) and (ii'), or components (i') (b) and (iii'), or components (i') (b), (ii') and (iii').

11. The process of claim 1, wherein coating layer B' is a transparent or a visually opaque coating layer.

12. The process of claim 1, wherein coating composition B is applied to coating layer A' when at least 50 wt. % of the volatiles of coating composition A are still present in coating layer A'.

13. The process of claim 1, wherein coating composition B is applied within 10 to 600 seconds of the application of coating composition A.

25 14. The process of claim 1 being carried out in the context of an industrial mass production coating process.

\* \* \* \* \*